

(No Model.)

2 Sheets—Sheet 1.

H. FRASCH.

REFINING CANADIAN OR SIMILAR PETROLEUM OILS.

No. 487,119.

Patented Nov. 29, 1892.

FIG. I.



FIG. II.



Attest:

Geo. T. Smallwood.  
Jas. K. McCathran.

Inventor:

Herman Frasch  
by Chas. J. Hedrick  
his attorney

(No Model.)

2 Sheets—Sheet 2.

H. FRASCH.

REFINING CANADIAN OR SIMILAR PETROLEUM OILS.

No. 487,119.

Patented Nov. 29, 1892.

FIG. III.



Attest:

Geo. T. Smallwood.  
Jas. K. McCathran

Inventor  
Herman Frasch  
Chas. J. Hedrick  
his attorney

# UNITED STATES PATENT OFFICE.

HERMAN FRASCH, OF LONDON, CANADA, ASSIGNOR TO THE SOLAR  
REFINING COMPANY, OF OHIO.

## REFINING CANADIAN OR SIMILAR PETROLEUM-OILS.

SPECIFICATION forming part of Letters Patent No. 487,119, dated November 29, 1892.

Application filed February 15, 1888. Serial No. 284,131. (No specimens.)

*To all whom it may concern:*

Be it known that I, HERMAN FRASCH, a citizen of the United States, residing at London, in the Province of Ontario, Canada, have invented certain new and useful Improvements in the Process of Refining Canadian and Similar Petroleum - Oils, of which the following specification is a full, clear, and exact description.

10 This invention relates to the treatment of Canadian and similar petroleum—such, for example, as that found at Lima, in Ohio. This oil requires a different treatment from the ordinary American oil, because of the sulphur compounds which it contains and which give it its penetrating disagreeable odor and render it unfit for burning in lamps unless deprived of said compounds. The sulphur is present in these oils in considerable proportions—say, upward of one-half of one per centum, ( $\frac{1}{2}$  of 1%), mostly in chemical combination, and some, at least, of the sulphur compounds are essentially different from those which occur in other oils and are retained with great tenacity. These peculiar sulphur compounds have received among the workers in the oils of this class the suggestive name of "skunk." To deprive these oils of their peculiar sulphur compounds or skunk is the 30 object of the present invention.

15 The large proportion of sulphur will generally distinguish Canadian and similar skunk-bearing petroleum from other oils; but a further distinction may be found in the nature of the sulphur-containing bodies therein. They give to the oils the property of dissolving lead oxide, (litharge.) So far as I am aware, no mineral oil, whether undistilled or distillate other than Canadian or similar skunk-bearing petroleum possesses this property of dissolving litharge. Ordinary petroleum can be made to dissolve litharge by the addition to said oil of a fat acid—such as oleic acid or rosin; but the Canadian or skunk-bearing petroleum will dissolve lead oxide (litharge) without such addition. Further, the skunk-bearing oil has a peculiar bad odor, which disappears on saturating the oil with lead oxide. On precipitating the lead from such solution by means of sulphur the bad odor does not reappear, neither does the oil regain the property of dissolving lead oxide. On distillation,

however, of the oil from which the lead has been precipitated, as just described, the malodor reappears, and the oil will again dissolve lead oxide, showing that the skunk remained even after the malodor disappeared. The malodor also reappears on burning and the lamp-chimneys become smoked. Moreover, while the sulphur existing in the oil as skunk is not removed by treating the oil with sulphuric acid and alkali (which treatment will remove practically all the sulphur existing in Pennsylvania oil) it is also true that after the removal of the skunk from Canadian and similar petroleum by the present invention there yet remains in said petroleum (now become sweet and incapable of dissolving lead oxide even after redistillation) sulphur in such form or forms that a repeated application of the skunk-removing process fails to eliminate it or materially to reduce its proportion, while it can be separated almost entirely by treatment with sulphuric acid. Skunk-bearing oil therefore is radically different from other mineral oils in respect to the sulphur bodies therein, said bodies giving to the skunk-bearing oil peculiar properties, as hereinbefore mentioned, and being not removable by the refining means in common use, which do remove the sulphur from American petroleum, while at the same time means efficient to remove skunk do not take out sulphur bodies removable by said refining means in common use on American oil, so that the utility of certain reagents or modes of treatment in desulphurizing other mineral oils is no proof of an ability to remove the skunk of Canadian and similar petroleum, nor does an ability to remove skunk constitute proof of a given process being capable of taking the place of the ordinary means of desulphurizing oil.

Heretofore it has been customary in Canadian refineries (and the same treatment has been employed in parts of the United States) to take the burning-oil distillate which has been subjected to the action of sulphuric acid and washed with water and to treat the same with a solution of plumbate of soda in order to deodorize it, and then to add sulphur in powder in order to restore the color which the plumbate solution has turned to a yellow or brown and cause the precipitation of the lead,

leaving the oil above it white and clear. The solution of soda settles to the bottom. The objections to this old deodorizing process are twofold: First, an excess of sulphur is liable to be added in the second stage, which is injurious to the oil, and, secondly, the treatment is not thorough, for it does not remove the sulphur compounds or skunk, but only renders the same inodorous and incapable of further uniting with the lead oxide of the plumbate solution. On distillation the sulphur compounds in the oil again become malodorous and the oil is discolored by the addition of the plumbate of soda solution.

15 In a prior application filed February 21, 1887, and officially serially numbered 228,403, (on which Patent No. 378,246 was granted me February 21, 1888,) I have described a process not open to these objections for refining 20 oil of the Canadian or Lima class by distilling the same with suitable oxides or compounds mixed with or dissolved in the oil under treatment. The present invention is, as it were, a supplement to or complement of 25 that process. I have discovered that the refractory sulphur compounds or skunk of Canadian and similar oils are decomposed by the metallic oxides or compounds without necessarily having such an oxide or compound 30 dissolved in or mixed with the oil in distillation by subjecting the vapors after leaving the liquid oil to the action of a suitable liquid holding in solution or solution and suspension one or more of the said oxides or their compounds. The vapors may be brought into 35 contact in any ordinary or suitable way with the liquid holding in solution or solution and suspension one or more of the oxides or compounds. The vapors may bubble through a 40 body of the liquid, or they may pass through a shower or spray of the same, or they may come in contact with the liquid in both these or in other ways.

In my divisional application, Serial No. 45 378,818, filed January 23, 1891, I have claimed that process or improvement which consists generally in subjecting the vapors of skunk-containing petroleum after leaving the oil in distillation to the action of suitable oxides 50 or compounds, for it is possible (although much less effective) to employ oxides or compounds otherwise than in solution or solution and suspension in a suitable liquid, and there are advantages incident to the carrying on of 55 the purification outside the oil in distillation which are not restricted to the use of a liquid, as above set forth, although very great and important special advantages attend such use.

Suitable oxides are those of the more 60 mon heavy metals which give up their oxygen with comparative readiness, and are generally those of metals which form sulphides convertible into oxides by roasting and oxidation. The oxides of lead, bismuth, cadmium, mercury, copper, and silver are well suited to the purpose, also binoxide of manganese, except for the difficulty of revivifica-

tion; but the ferric, stannic, and antimonic oxides, cuprous oxide, and the oxides of nickel, cobalt, and zinc are less energetic and are 70 more useful in connection with those first mentioned, among which is to be included manganese binoxide, than when used alone. The lower oxides of manganese and the oxides of palladium and rhodium may be used. 75 The oxides of manganese are more useful when employed in connection with lead oxide than when used alone.

Suitable compounds are the readily-decomposable oxygen compounds—such, for example, as the carbonates of metals—which give up their oxygen with comparative readiness and the oxygen salts in general of metals which are precipitated by hydrogen sulphides in acid solutions, such as the manganates, 80 chromates, borates, sulphates, and the like of said metals.

Suitable liquids are those of an oily or resinous nature, and especially those oily liquids which have the property of dissolving the 90 metallic oxide or oxides employed—such, for example, as the impure or skunk-containing Canadian or Lima oil itself of preferably higher boiling-point than the oil which is vaporized and subjected in vapor form to the 95 action of the oxides or decomposable oxygen compounds dissolved in or mixed with said liquid. The vapors from one still may in fact be passed through the liquid in another still, in which latter the oil under treatment is 100 mixed with or holds in solution one or more suitable metallic oxides or compounds. In employing an oily solvent liquid in whatever way in connection with the oxide or compound which attacks the skunk the effectiveness of the process is much increased by supplying and maintaining the oxide or compound in excess of the solvent capacity of 105 said liquid, so as to have the solution saturated with undissolved oxide or compound mixed 110 therewith in solid form, for the oxide is in the most active condition when dissolved, and as the reaction with the sulphur compounds or skunk takes place metal is precipitated 115 from the solution in chemical combination with sulphur and fresh oxide or compound will dissolve if it has been mixed with the previously-saturated solution. The vapors to be treated in accordance with the present 120 invention can be generated from the crude oil or from any desired distillate. The purification or refining is, however, specially intended for burning-oil having a boiling-point of 212° Fahrenheit or over. I have also discovered 125 that the refining operation, as well in carrying on the purification outside the liquid in or from which the vapors have been generated as in proceeding according to the specification of my aforesaid patent, is improved in respect to the rapidity with which it can 130 be carried on by the use in connection with the metallic oxides or compounds of one or more of the acid hydrocarbons, such as oleic acid, stearic acid, margaric acid, colophonic

acid, (rosin,) and other fatty or resinous acids. The acid may be mixed with the oxide or compound or be in chemical combination therewith. In fact all the metal employed 5 could be in the form of a colophonate, stearate, oleate, or the like. The liquid condensed from the vapors which have thoroughly been brought into contact with the oxide or compound, so as to give it opportunity to act 10 upon all the sulphur compounds or skunk, will stand the plumbate-of-soda test. I find, however, that the condensed liquid or distillate purified from skunk, although it will stand the plumbate-of-soda test, yet contains 15 sulphur compounds, which I believe to be peculiar to oil treated in this way and which impair the value of the oil by causing a chimney-deposit when burned in a lamp. These products, like the similar or identical ones 20 from distilling the oil with the purifying oxide or compound mixed with or dissolved in the same, are essentially different from skunk and are, as I have discovered, removable by treatment with sulphuric acid, washing with 25 water, and neutralizing, as customary in refining American petroleum.

The metallic sulphur compounds which are formed by the reaction with the sulphur-containing impurities of the vapors, as above set 30 forth, can be revivified by roasting and oxidation and these revivified residues can be employed successfully to treat new vapors of Canadian or Lima or similar skunk-bearing oil.

In order the better to enable those skilled 35 in the art to practice the invention, the following detailed description is given, reference being had to the accompanying drawings, which form part of this specification, it being understood that the invention is not 40 restricted to the precise numbers given nor to other details of the process, nor to apparatus, but that these are described by way of illustration and example.

In the drawings, Figure I is a sectional view 45 of an oil still and purifier suitable for use in carrying the invention into effect. Fig. II is a similar view of a slightly-modified form of the same apparatus, and Fig. III is a similar view of another form of apparatus.

50 Referring to Figs. I and II, an ordinary still A is provided with a column B, which has baffle-plates or trays and stirrers, as common, or at least known, in various chemical arts. In Fig. I the baffle-plates 2 are in the form of circular disks, which are mounted horizontally 55 on an upright central shaft 3, and the baffle-plates 4 are in the form of rings fastened to the walls of the column B and projecting inward between the disk plates 2. In Fig. II the trays 5 are fastened to the walls of the column, and the openings for the passage of the vapors are formed at the opposite sides of alternate trays, and the shaft 6 is provided with stirrers which dip into the trays. In both figures the top of 65 the still A is connected by a vapor-pipe 7 with the column B, and at the top of the latter there is a pipe 8 for conveying the purified vapors

to the condenser. (Not shown). A pipe 9 leads from the base of the column B to the pump C and a pipe 10 from the said pump 70 C to the top of said column. The shafts 3 and 6 are rotated by bevel-gear, and the column B, which rests on a pillar 11, is heated by the products of combustion from the fire-chamber D under the still on their way to the 75 chimney E. The column B should be of such size as to bring the vapors sufficiently into contact with the purifying material. If the still be such as commonly used to distill a charge of one hundred barrels of oil, the column B may be, say, ten feet high and four feet in diameter, with the baffle-plates or trays about six inches apart.

In operation the still is charged with, say, one hundred barrels of oil composed of, say, 85 fifteen per centum of heavy oil of from 36° to 39° Baumé, and the remainder burning-oil distillate boiling at 212° Fahrenheit or over. The column is supplied with, say, five barrels of heavy impure or skunk-bearing Canadian or similar oil mixed with, say, one barrel of rosin, five hundred pounds of plumbic oxide, (litharge,) one thousand pounds of cupric oxide, (black oxide,) and one thousand pounds of plaster-of-paris, the oxides and plaster being finely ground and bolted. The rosin and part of the oxides dissolve in the oil and the rest of the oxides and plaster are kept in suspension therein. The oil, with the matter in solution and suspension therein, flows over 100 the baffle-plates or trays, which trays become filled, and collects in the bottom of the column B. After or before the oil is introduced the pump is started which draws off through the pipe 9, the oil holding the oxide in solution and suspension therein and returns it to the top of the column B through the pipe 10. The shaft 3 in the column is also rotated. The rotation of the disks 2, Fig. I, throws the liquid and solids off onto the rings 4, from which 105 they descend to the next disk by gravity, the flow of the liquids being sufficient to sweep away the solid particles; but, if desired, mechanical devices or scrapers could be employed to sweep or scrape the surfaces of the 110 baffle-plates, as well known in chemical apparatus, wherein gases or vapors are to be brought into contact with liquids holding solid particles in suspension therein. The rotation of the shaft 3 also keeps the material stirred up 115 in the bottom of the column B by means of an ordinary blade or paddle. The rotation of the shaft 6, Fig. II, keeps the material stirred up in the trays 5 and at the bottom of the column. The still A and the column B 120 being charged and the pump C and shaft 3 (or 6) in column B being started, the still A and column B are heated, the former to evaporate the burning-oil therein and the latter to prevent or diminish the condensation of the 125 vapors from the still. The vapors pass through the pipe 7 into the lower part of column B, through which they then pass upward, and are in their passage brought into intimate con-

130

tact with the liquid holding the oxides in solution and suspension, said liquid, with the oxides, flowing in the opposite direction over the baffle-plates or trays and falling from one to the other through the rising vapors. The vapors escape by the pipe 8 to the condenser. The passage of the vapors through or over the liquid enables the oxides to act on the skunk in said vapors with the formation of metallic sulphur compounds which remain in the liquid and certain new bodies which pass off with the vapors. A constant stream of the oil having the oxides dissolved and suspended therein is introduced at the top of the column B and drawn off at the base. The liquid drawn off is returned to the column, the whole or a portion of the precipitated or solid matter in suspension being removed and replaced by fresh oxides at each round or from time to time. As the metal of the oxides in solution combines with the sulphur of the skunk and becomes insoluble fresh oxide enters the solution, the same being supplied from the matter in suspension. The still is or may be supplied continuously or from time to time with the burning-oil distillate.

It is not necessary to have the column B heated otherwise than by its proximity to the still A and the passage through it of the vapors from said still; but in that case the condensed vapors must be taken care of either by returning them to the still or otherwise. If solid matter is allowed in the still either by entering in that state from the column B or by precipitation in the still, the latter should be provided with an agitator to keep it from settling.

The plumbic or the cupric oxide could be used alone—say thirty-three hundred pounds of plumbic oxide or twelve hundred pounds of cupric oxide—or one or both could be replaced by or used in connection with another or others of the specified agents. The plaster and the rosin may be omitted.

It is not necessary to use heavy oil in the purifier-column, although such oil is preferable to a lighter petroleum, because it does not volatilize in the column; nor need the oil in the said purifier-column contain the sulphur compounds which enable it to dissolve the oxides, for the solubility of the oxides might be secured by other means—such as the use of a fat acid—or the oxides, if simply held in suspension in an oily menstrum not originally a solvent of the oxides, will become dissolved by reason of the skunk brought over by the vapors from the still; nor need petroleum be used at all, as rosin alone would answer.

According to another plan of working (see Fig. III), the still A is provided inside with a large pipe F, which communicates with the interior of the still through the opening 15 and also with a small column G, such as used in rectifying alcohol on top of the still, and with a small vessel or receiver 16 inside the still. A steam-injector or steam-jet aspirator and

compressor H sucks the vapors from the upper part of the still A and forces them through the pipe F into the bottom of the column G. The injector H also forces into the pipe F and among the vapors therein the purifying oxide or compound finely divided and dissolved in or mixed with an oily liquid. As shown, there is a reservoir K, provided with a stirrer 17, from which the injector H draws a supply of oxide or compound in suspension or in solution and suspension in the oily liquid. More or less of the oxide is forced with the vapors into the column. What does not so pass is carried into the small vessel or receiver 16, the object of which is to keep the sediment from the bottom of the still. This material could be allowed to run into the still; but in that case the latter should have an agitator, or it could be discharged outside of the still to be returned or otherwise disposed of. The column G has an overflow at the bottom, which discharges into the receiver 16. The oil or condensed vapor in this receiver is volatilized again and passes in vapor form into the pipe F and then into the column G. The large pipe F may have an opening into the vapor-space at each end, so as to circulate the vapors through the pipe as well as force them into the column G. The steam-jet to force the vapors could be used in the arrangements described with reference to Figs. I and II. Other modes of bringing the vapors into contact with the purifying agents have been indicated in the first part of this specification.

The larger the proportion of skunk in the oil the more thoroughly should the vapors be brought into contact with the purifying agents, and if the process is carried on by batches—that is, without a constant renewal of the oxide or compound—care should be taken to have the amount of purifying agent larger than necessary to decompose all the skunk. The weight of oxides given would be ample for one hundred barrels of oil containing about one-half of one per centum of sulphur.

The vapors from the purifying apparatus are received in a condenser (not shown) and the condensed liquid is washed with sulphuric acid, or it may be used without such washing.

The solid sulphur-containing residue from the above operation or from an analogous operation is roasted and oxidated and after grinding and bolting is used like fresh oxide.

In order to revivify the purifying agent or agents, the solid residue is or ordinarily would be separated by straining or otherwise from the oily or resinous liquid with which it is mixed and is then thrown into the front part of a roasting-furnace a portion at a time and ignited. The oil adhering, in connection with the sulphur and metal, furnishes all the heat necessary for roasting. The air will supply the oxygen, so as to effect the revivification at one operation. As each fresh portion is added, the portions previously introduced are

- pushed back until the whole charge has been transferred to the furnace. The mass becomes red-hot and is thoroughly roasted and oxidized. The fine division of the powder and its composition insure a perfect and quick roasting. It is stirred until below red heat and is then discharged to be reground for use again. The oily or resinous liquid is used again with fresh purifying agents.
- 10 I do not claim herein the apparatus described. It forms the subject of my application, Serial No. 289,746, filed November 1, 1888; nor do I claim herein the revivification of the residue of the revivified residues, as such matter forms the subject of my application, Serial No. 284,830, filed September 7, 1888; but the use of the revivified residues, as herein described, is included in the present invention.
- 20 The expression "vaporizing the oil and subjecting the same to the action" as employed in the second, fourth, and fifth clauses of claims following is intended to apply as well to the action which occurs within the oil when the latter is distilled with the purifying agent dissolved therein or mixed therewith as to an action on the oil vapors after they have been given off from the body of the liquid oil undergoing distillation.
- 30 The advantages which are secured by the carrying on of the process of purification of the vapors of distillation outside the oil in or from which the same have been generated are not confined to the use of a liquid solvent, but to a greater or less degree extend to the use of the oxides in a dry state, and this general feature of my invention—namely, the carrying on of the purification outside the liquid in or from which the vapors have been generated—is made the subject of my divisional application, Serial No. 378,818, filed January 23, 1891.
- I claim herein as my invention or discovery—
- 45 1. The process of removing the sulphur compound termed "skunk" from Canadian and similar petroleum, which consists in vaporizing the oil and subjecting the vapors after they are given off from the body of the oil to the action of an oily or resinous liquid holding in solution or solution and suspension one or more metallic oxides soluble in said oil, including the decomposable compounds of such oxides, and condensing such purified vapors, substantially as described.
- 50 2. The process of removing the sulphur compound termed "skunk" from Canadian and similar petroleum, which consists in vaporizing the oil and subjecting the same to the action of a solution in an oily or resinous liquid composed of one or more metallic oxides soluble in said oil, including the decomposable compounds of such oxides, and maintaining an excess of the soluble but as yet un-
- 65 dissolved purifying agent in suspension in said solution, whereby the said liquid is kept saturated, substantially as described.
3. The process of removing the sulphur compound termed "skunk" from Canadian and similar petroleum, which consists in vaporizing the oil, subjecting the vapors after they are given off from the body of the oil to the action of films, showers, or sprays of an oily or resinous liquid holding in solution or solution and suspension one or more metallic oxides soluble in said oil, including the decomposable compounds of such oxides, and condensing such purified vapors, substantially as described.
- 70 4. The process of removing the sulphur compound termed "skunk" from Canadian and similar petroleum, which consists in vaporizing the oil and subjecting the same to the action of purifying material, composed of or containing one or more of the metallic oxides soluble in said oil, including their decomposable compounds, and one or more fatty or resinous acids, such as oleic, stearic, margaric, colophonic acids, substantially as described.
- 75 5. The process of removing the sulphur compound termed "skunk" from Canadian and similar petroleum, which consists in vaporizing the oil and subjecting the vapors to the action of a metallic oleate, colophonate, or other metallic salt of a fatty or resinous acid, substantially as described.
- 80 6. The process of removing the sulphur compound termed "skunk" from Canadian and similar petroleum, which consists in vaporizing the oil and subjecting the vapors after they are given off from the body of the oil to the action of an oily or resinous liquid containing said sulphur compound termed "skunk," and one or more metallic oxides soluble in skunk-bearing oil, including the decomposable compounds of such oxides, and condensing such purified vapors, substantially as described.
- 85 90 95 7. The process of removing the sulphur compound termed "skunk" from Canadian and similar petroleum, which consists in vaporizing the oil and subjecting the vapors after they are given off from the body of the oil to the action of an oily or resinous liquid holding in solution or solution and suspension one or more metallic oxides soluble in said oil, including their decomposable compounds, condensing such purified vapors, and washing the condensed liquid with sulphuric acid, substantially as described.
- 100 In testimony whereof I have signed this specification in the presence of two witnesses.

HERMAN FRASCH.

Witnesses:

J. W. VAN DYKE,  
W. B. RICHIE.

It is hereby certified that in Letters Patent No. 487,119 granted November 29, 1892, upon the application of Herman Frasch, of London, Canada, for an improvement in "Refining Canadian or Similar Petroleum Oils," an error appears in the printed specification requiring correction as follows: In line 61, page 5, the word "composed" should be stricken out; and that the Letters Patent should be read with this correction therein that the same may conform to the record of the case in the Patent Office.

Signed, countersigned, and sealed this 24th day of January, A. D. 1893.

[SEAL.]

CYRUS BUSSEY,  
*Assistant Secretary of the Interior.*

Countersigned:

W. E. SIMONDS,  
*Commissioner of Patents.*